

## UNITED STATES PATENT OFFICE

JAMES ELIOT BOOGE, OF WILMINGTON, DELAWARE, ASSIGNEE TO E. I. DU PONT DE NEMOURS & COMPANY, OF WILMINGTON, DELAWARE, A CORPORATION OF DELAWARE

STABLE HOMOGENEOUS NITROCELLULOSE-DRYING OIL MIXTURES AND PROCESS OF MAKING SAME

No Drawing.

Application filed October 8, 1925. Serial No. 61,264.

This invention relates to a process of producing a homogeneous mixture of a drying oil compound with nitrocellulose, and to the nitrocellulose mixture resulting from such process. More particularly the invention comprises, as a new process, oxidizing a drying oil, as by blowing it with air, until a test shows that it is completely and easily miscible with nitrocellulose, at which time its iodine number will be substantially less than what it was originally, and then mixing it with the nitrocellulose; and, as a new product, the homogeneous mixture of nitrocellulose and oxidized, or blown, drying oil, with or without other modifying agents and/or thinners.

For various purposes in the arts it is desirable to combine vegetable oils in various proportions with nitrocellulose or with a solution of nitrocellulose in solvents. It is known that various non-drying oils can be used in this way and that such oils as castor may be incorporated with nitrocellulose with a fair degree of ease. However, when attempts have been made to use drying oils such as linseed oil or chinawood oil, it has been found that the oil tends to precipitate the nitrocellulose when the solvent evaporates, and that permanent mixtures can be obtained only if an excessive amount of nitrocellulose solvent is used and if in addition one of the principal ingredients, that is, either the oil or the nitrocellulose is present in relatively small proportions. When, for instance, the attempt has been made to incorporate any considerable proportion of raw or boiled linseed oil with the nitrocellulose, it has been found that even though an excessive amount of solvent, is used, the oil tends to separate on standing or when the solvent evaporates, so that a clear homogeneous film cannot be obtained.

Moreover it has been found that even though used in excessive amounts the only nitrocellulose solvents which are effective in this case are the more expensive high-boiling solvents such as amyl acetate, etc. Therefore, because of the small amount of oil which can be permanently combined with nitrocellulose, and, further, because of the high price and

large amount of solvent required to hold the mixture together, the practical result has been that up to this time mixtures of nitrocellulose with substantial proportions of drying oils have not been available to the nitrocellulose industries.

Now I have discovered that all of these difficulties may be avoided and a permanent mixture obtained, if the drying oil before incorporation is subjected to a suitable blowing treatment with air or oxygen such as is more particularly described below. By this treatment the oil may be rendered miscible with the nitrocellulose practically in all proportions, and the mixture once formed is permanent and no separation of oil from nitrocellulose takes place either on standing or after the solvent has evaporated.

The pyroxylin-oil solution thus formed may be diluted or thinned as desired to reduce the viscosity, and I find that because of the complete compatibility of the blown drying oil with the nitrocellulose the diluent need not be a solvent for nitrocellulose but may include such non-solvents as turpentine, benzol, xylol, etc., as well as mixtures of such liquids. However, the diluent may be varied over a fairly wide range of liquid nitrocellulose solvents and non-solvents to suit the particular purpose required.

In preparing the oil for use according to my preferred process, I may start with linseed, chinawood, perilla or other drying oil. This is heated to a suitable temperature and subjected to blowing with air. The air is forced up through the oil preferably in fine bubbles. There results a drop in the iodine number of the oil, accompanied by an increase in the viscosity or body. The blowing is continued until it is found on test that the oil is completely miscible with pyroxylin jelly.

In the examples given below the oil used was linseed which had been blown at 100° C. for about 4 hours and was then found on test to be completely compatible with pyroxylin jelly. The nitrocellulose used is of the type usually used in pyroxylin mixtures and contained about 12% nitrogen. The solvent mixture may be varied widely, but in general

there should be sufficient active nitrocellulose solvents present to yield a clear film. In the examples below pyroxylin solution was made up containing 16 oz. of nitrocellulose per gallon. The solvent used was of the following composition:

10 butyl acetate, 2%  
ethyl acetate, 18%  
alcohol, 20%  
benzol, 60%

*Example 1*

25 parts blown linseed oil  
15 24 parts 16-oz. pyroxylin jelly (12.5% N. C.)  
51 parts benzol

*Example 2*

28 25 parts blown linseed oil  
40 parts 16-oz. pyroxylin jelly  
35 parts benzol

*Example 3*

25 33 parts blown linseed oil  
33 parts 16-oz. pyroxylin jelly  
17 parts turpentine  
17 parts benzol

30 Where the nitrocellulose composition is to function as a plastic, the proportion of drying oil used will be smaller than in the above examples, the exact amount depending upon the particular use of the composition and the presence or absence of other softening agents.

35 The mixture illustrated in the above examples can be used for various purposes with suitable variation in the content of thinner, as for instance in the manufacture of artificial leather, films, etc.

40 The term "drying oil", as used in the claims, covers linseed, chinawood, perilla, and other oils of the drying type, but does not cover semi-drying oils, such as cottonseed oil and olive oil; and in order clearly to distinguish between these two types, which are materially 45 different in their action for the purposes of this invention, I define drying oils as those having an iodine number of not less than 120.

50 As many apparently widely different embodiments of this invention may be made without departing from the spirit thereof, it is to be understood that I do not limit myself to the above embodiments, except as indicated in the appended claims.

55 I claim:

1. The process of making a permanent mixture of nitrocellulose and a drying oil which comprises blowing the hot oil with an oxidizing agent until said oil is completely miscible 60 with pyroxylin jelly, and then mixing the blown oil with nitrocellulose.

65 2. The process of making a permanent mixture of nitrocellulose and a drying oil which comprises blowing the hot oil with air until 70 said oil is completely miscible with pyroxylin jelly, and then mixing the blown oil with a solution of nitrocellulose in a liquid which is also a solvent for the blown oil.

lin jelly, and then mixing the blown oil with nitrocellulose.

3. The process of making a permanent mixture of nitrocellulose and a drying oil which comprises blowing the hot oil with air until 70 said oil is completely miscible with pyroxylin jelly, and then mixing the blown oil with a solution of nitrocellulose in a liquid which is also a solvent for the blown oil.

4. In the process of making a permanent mixture of nitrocellulose and a drying oil, the step which comprises heating the oil, and blowing the hot oil with air until it has become so miscible with nitrocellulose as to form therewith a permanent homogeneous mixture and then mixing the blown oil with the nitrocellulose.

5. The process of making a permanent mixture of nitrocellulose and a drying oil which comprises heating the oil, blowing the hot oil with air until it has become completely and permanently miscible in the desired proportion of pyroxylin jelly, and then mixing the blown oil with nitrocellulose.

6. A process as claimed in claim 5 in which 90 the blown oil is mixed with nitrocellulose in the presence of a common solvent.

7. The process of making a mixture of a drying oil and nitrocellulose which comprises blowing the oil with air while maintaining 95 the oil at a temperature of about 100° C. until the oil has become miscible in the desired proportion of pyroxylin jelly, and then mixing the oil with nitrocellulose in the presence of a common solvent.

100 In testimony whereof I affix my signature.  
JAMES ELIOT BOOGE.

105

110

115

120

125

130